

## UNITED STATES PATENT OFFICE

TURE ROBERT HAGLUND, OF STOCKHOLM, SWEDEN

## PROCESS FOR PRODUCING METALS AND ALLOYS

No Drawing. Application filed July 31, 1924, Serial No. 729,354, and in Sweden October 8, 1923.

The present invention relates to a process for producing metals and alloys, which makes it possible to obtain an improved regulation of the quantity of metals to be alloyed with a metal or alloy as compared with the results of hitherto known processes for the production of metals and alloys in electric furnaces. The chief object of the invention is a process for reducing metals and alloys with a low percentage of carbon but the process may in many cases also be used with great advantage for the production of metals and alloys with higher percentages of carbon. In the hitherto known electro-metallurgical processes where carbon or carboniferous reducing agents are used, the ores or other raw materials, from which the metals or alloys are to be produced, are reduced either directly with carbon or, as is the case when producing pig iron, partly with carbon and partly with the carbon-mono-oxide containing gases formed in the process. To produce a product with low percentage of carbon by such means has as a rule hitherto not been possible. Instead it has been necessary, in order to get such a product with low percentage of carbon, to refine the product with great costs.

The present process renders it possible to produce directly metals and alloys with low percentage of carbon, even such metals and alloys that will easily absorb carbon. This object is attained by reducing the ore or the like entirely or mainly not directly but indirectly with carbon or carboniferous reducing agents. A suitable mixture of oxidiferous material and carboniferous reducing agents are formed into bricks or lumps of rectangular or other form which lumps are charged in a furnace together with the ore or the like from which the metal or alloy is to be produced. The ingredients for the bricks or lumps should be pulverized and intimately mixed. The specially prepared material in the lumps will first be reduced in the furnace and the metal or the like thus produced will in its turn act as a reducing agent upon the other material.

The oxidiferous materials in the bricks or lumps must be of such quality that, when it is reduced by carbon, such elements, alloys or

carbides are formed, as will have a reducing action upon the raw material proper for the metal or alloy to be produced. For example the following oxides may be used as an ingredient in the bricks or lumps, namely aluminum oxide, magnesium oxide, barium oxide, calcium oxide, silica, manganese oxide, boric acid, chrome oxide, zinc oxide and others. Each of these oxides or a mixture of two or more of them may be used in the bricks or lumps, different sorts of which may be used together. It may be advantageous to use special agents in the process for getting a suitable consistency and melting point of the slag and such agents may be mixed into the bricks. As a rule, however, it will be more suitable to add separately such agents, that are not to be influenced by the reducing carboniferous agents. These agents which naturally must be chosen with due regard to the nature of the oxidiferous materials in the bricks or lumps and of the slag forming ingredients in the other materials may consist of lime, quartz, fluor-spar, sulfides such as CaS and others. As reducing agents in the bricks or lumps one or more carboniferous materials may be used such as charcoal, graphite, anthracite, coal, lignite, coke, lignite coke (or dust or grits of said carboniferous materials), peat, sawdust and others. If a carboniferous material other than a coke is an ingredient in the bricks or lumps these may be previously heated to make the fuel to coke. This will also make the bricks hard and porous. A binding agent for the content of the bricks or lumps may, if necessary, be used such as the usual agents for brick-making namely tar, marl, lime-water, clay, water-glass, sulphite, waste lye and others. When bricks of special strength are required they may be previously sintered or burnt.

Metals or alloys which with great advantage may be produced by the present process are for example, chromium, iron, manganese, titanium, vanadium, tungsten, molybdenum and alloys containing the metals named.

For the production of ferro-chromium from the commercial chromium oxide ore (chromite) or for the production of ferro-chromium alloys with lower percentage of

chromium, for example rustless iron and steel, out of mixtures of such ore and iron ore (or metallic iron), it is suitable to use 5 bricks or lumps containing one or more oxides such as aluminum oxide, calcium oxide or magnesium oxide. Upon the reduction of the bricks in the furnace in this case aluminum, calcium or magnesium metal will be produced (or, according to the percentage 10 of carbon in the bricks, carbides, for example calcium carbide), which metals (or carbides) will rapidly reduce the chromium oxide ore charged together with the bricks or lumps. Whereupon aluminum oxide, calcium oxide or magnesium oxide will again 15 be formed, which oxides are taken up in the slag. As suitable aluminum oxide containing raw material in the bricks or lumps may be used aluminum oxide, alundum, bauxite and others. As suitable magnesium oxide containing raw material may be used magnesite or dolomite and others, and as suitable calcium oxide containing raw material may be used limestone, burnt, lime, marl and 20 others. As the slag forming ingredients by reduction of chromite mainly will be aluminum oxide and magnesium oxide, the slag produced may be used for the brick-making. The temperature in the reduction zone of the 25 furnace will be higher than by the reduction of chromium oxide ore directly by means of carboniferous reducing agents, and the slag will accordingly be hotter and more easily tapped than by the hitherto used processes 30 for the production of ferro-chromium.

If the bricks are of high specific gravity it may in some cases be advantageous for easing the work of the furnace to add a part 35 of the reducing agents in the charge in the form of lumps of carbon material, for example lumps of charcoal. Only a small quantity of such charcoal will be needed if a specially high percentage of carbon in the alloy is not desired. An excess of chromium 40 oxide ore may be eventually added for the compensation of such additional charges of carboniferous material. It is however more convenient to use carboniferous reducing agents in the bricks or lumps of such quality 45 that light and porous bricks are formed, in which case no supplementary addition of carboniferous materials is needed.

By using a surplus of bricks in proportion 50 to the quantity of chromium oxide ore it will be possible to produce chromium alloys with for example a high percentage of aluminum. In this case a slag of low specific gravity 55 may suitably be used. As ingredients in the slag, effecting a low specific gravity of same may be mentioned calcium sulphide, aluminum sulphide, magnesium sulphide and magnesium oxide. These named sulphides may be brought into the slag by adding charges of material already containing 60 such sulphides, or additional charges may

be made of some other sulfidiferous material such as sulphide of iron, magnetic iron pyrite and others. These materials will during the process, for example by reaction with the metal reduced out of the bricks, form in 70 the furnace one or more of the light sulphides above mentioned, whereby the iron or other metal content in the sulfidiferous material is separated out.

If, however a chromium alloy with low 75 or no percentage of aluminum is to be produced by means of bricks or lumps containing aluminum oxide the content of chromium oxide ore in the charge is accordingly regulated so that aluminum metal reduced out 80 will wholly or substantially be oxidized through reaction with the chromium oxide ore. In this case it will be advantageous to work with a slag of comparatively high specific gravity, the reason for this being that 85 the reduction of the chromium oxide ore mainly will take place in the zone above the slag and accordingly a quicker reduction effected than will be the case if the chromium oxide first is solved in the slag from which 90 it must be reduced out.

Upon the reduction of bricks or lumps containing magnesium oxide or calcium oxide, the magnesium or calcium metal will be obtained in the form of gas which vastly facilitates 95 the reducing action on the ore. This appearance of the metal in the form of gas in the furnace will also take place to a great extent when aluminum metal is reduced out of bricks. The furnaces for the production 100 of chromium or chromium alloys with the described method may suitably be the usual furnaces of the carbide furnace type.

The production of other metals and alloys with the present method is effected in 105 a similar way to that described above with reference to the production of chromium alloys.

For the production by means of the present process of iron or steel it is especially 110 advantageous to determine the ingredients in the bricks or lumps and the rest of the charge in such a manner that the slag formed by the smelting has such quality as to be suitable for the production of cement. The working of the slag into cement may be 115 effected by means of the usual methods. By means of the present process it will thus be possible to produce as a by-product not only cement of the usual Portland composition but also more rapidly hardening aluminate cement and lime-aluminate cement. For the production of Portland cement the oxide containing raw material in the bricks or lumps may suitably consist of one or 120 more CaO containing materials such as lime-stone, marl or burnt lime and of clay, bauxite or other  $Al_2O_3$  containing material and if necessary also of quartz or other  $SiO_2$  containing material. For the production of 125

cement richer in aluminum oxide it will be best to use bauxite as an  $Al_2O_3$  containing raw material. The bricks or lumps are suitably made with use of lime-water, clay or cement as a binding agent. For this purpose a part of the cement obtained in the process may be used, thereby circulating it in the process.

If however, the production of cement slags is not desired, bricks may be used with a high percentage of silica such as for example quartz or sand. If the iron ore contains lime, bricks may be used which contain, besides reducing agents, mainly silica. In other cases slag-forming materials other than silica must as a rule also be added, either forming part of the bricks or being charged separate. Two or more sorts of bricks or lumps may be used, for example bricks containing one or more of the oxides of calcium, magnesium or aluminum and carboniferous materials together with bricks containing  $SiO_2$  and carboniferous materials. Slags such as for example calcium-silicates or manganese-silicates may also be used as oxidiferous ingredients in the bricks. In this case calcium-silicid or manganese-silicid will first be formed and these silicides thereupon reduce the iron ore. Aluminium silicates such as chamotte, clays and others may also be used as suitable raw materials for the bricks.

On account of the fact that the temperature in the furnace mainly is determined by the reduction temperature for the bricks, the products smelted by the process will reach a higher temperature than will be the case when producing for example pig iron in the usual way in an electric furnace. Thus the temperature will be sufficiently high even for the tapping of iron with low content of carbon.

If the bricks or lumps are used in excess of iron ore, the iron may be obtained with the metal reduced out of the bricks, for example silicon, manganese, aluminum, chromium and others. If however such amount of iron ore is used that a part of the iron oxide remains, unreduced in the charge, it is possible by the present method to obtain a product poor in carbon and other alloy ingredients. This product should however, as a rule, be subsequently treated in a special electric furnace for adjustment of the percentage of carbon and sulfur cleaning and so on. This subsequent treatment can however be made in much shorter time and will be much cheaper than the refining of pig iron.

The production of iron with the present process may if the iron ore mainly is in form of lumps be carried out in the usual electric shaft furnace. If the iron ore is finely granulated or pulverized it will be more advantageous to work in an electric furnace of the carbide furnace type.

For the production by the present method of metals and alloys with extremely low percentage of carbon, the quantity of carboniferous material in the bricks or lumps should as a rule be less than the quantity of carbon required for the complete reduction of the oxidiferous material in the bricks or lumps.

Having thus described my invention I declare that what I claim is:

1. A process for producing carbide-forming metals or alloys, which comprises reducing ores by fusing them in an electric furnace together with a quantity of reducing agent for the ores added in the form of lumps of material containing bauxite, a basic refractory oxide having a lower melting point than the ores and carbonaceous reducing agents.

2. A process for producing metals or alloys adapted to form carbides, which comprises reducing ores by fusing them in an electric furnace together with a quantity of reducing agent for the ores added in the form of lumps of material containing bauxite and carbonaceous reducing agents and lumps of material containing magnesium oxide material and carbonaceous reducing agents.

3. A process for producing ferro-chromium alloys, which comprises reducing chromite ore by fusing it in an electric furnace together with a quantity of carbonaceous reducing agents added for the greater part in the form of ingredients of lumps of material containing in addition to the carbonaceous agents a considerable amount of magnesium oxide.

4. Process for producing the elements with atomic number from 22 to 26 in the periodic system, or alloys containing at least one of said elements, which comprises preparing a charge containing an oxide of at least one of said elements and at least one oxide having a heat of formation equal to or higher than that of said first oxide; and carbon reducing agents in amounts insufficient for the reduction of more than a part of the whole oxide content; keeping in the unfused condition the oxide of the first named kind, keeping said oxide, compared with the last named kind, in less intimate contact with the reducing agents by adding a considerable part of the carbon reducing agents in the form of lumps, said lumps besides the reducing agents containing mainly an oxide of the last named kind; and reducing the oxide of the first named kind by fusing the charge in an electric furnace.

5. Process of producing the elements with atomic number from 22 to 26 in the periodic system, namely titanium, vanadium, chromium, manganese or iron, or alloys containing at least one of said elements, which comprises preparing a charge containing an oxide ore of at least one of said elements and at least one of the oxides of aluminum, magnesium and calcium; and carbon reducing agents in amounts insufficient for the reduc-

120  
125  
130

tion of more than a part of the whole oxide content; keeping in the unfused condition the oxide of the first named kind, said oxide, compared with the last named kind, being kept in less intimate contact with the carbon material by adding at least a considerable part of the carbon reducing agents in form of lumps which besides the reducing agents mainly contain a considerable amount of at least one of the oxides of aluminum, magnesium and calcium; and reducing the oxide of the first named kind by fusing the charge in an electric furnace.

6. Process for producing ferrochromium alloys, which comprises preparing a charge containing chromite ore and material containing at least one of the oxides of aluminum, magnesium and calcium, and carbon reducing agents in amount insufficient for the reduction of the whole content of oxides of iron and chromium; keeping in the unfused condition the chromite compared with the material containing at least one of the oxides of aluminum, magnesium and calcium, 20 said chromite being kept in less intimate contact with the carbon material by adding at least a considerable part of the carbon material in the form of lumps, said lumps besides the carbon material mainly containing at least one of the oxides of aluminum, magnesium and calcium; and reducing the oxides of iron and chromium out of the chromite by fusing the charge in an electric furnace.

7. Process for producing chromium-alloyed iron or steel, which comprises preparing a charge containing chromite ore and iron and a material containing at least one oxide which has a higher heat of formation than that of chromium oxide; and carbon reducing agents in amounts insufficient for the reduction of more than a part of the whole oxide content; keeping in the unfused condition the chromite and the iron, said materials, compared with the oxide of the higher 40 heat of formation, being kept in less intimate contact with the carbon material by adding at least a considerable part of the carbon material in form of lumps, which besides the carbon material mainly contain an oxide of the last named kind; and reducing the oxide in the chromite ore by fusing the charge in an electric furnace.

8. Process of producing chromium-alloyed iron or steel, which comprises preparing a charge containing chromium oxide ore, iron ore, material containing at least one of the oxides of aluminum, magnesium and calcium, and carbon reducing agents in amounts insufficient for the reduction of the whole 55 content of oxides of iron and chromium, keeping the chromium oxide in the unfused condition, said oxide, compared with the last named kind of oxides, being kept in less intimate contact with the carbon material by adding a portion of the reducing agents as

lumps of carbon material and another portion in form of lumps which, besides the carbon material, mainly contain a considerable amount of at least one of the oxides of aluminum, magnesium and calcium, and reducing the oxides of iron and chromium by fusing the charge in an electric furnace.

In testimony whereof I affix my signature.

TURE ROBERT HAGLUND.

75

80

5

90

95

100

105

110

115

120

125

130